

Jan. 11, 1944.

R. B. PORTER

2,338,781

METHOD AND APPARATUS FOR CONTINUOUSLY CASTING METALS

Filed April 24, 1942

2 Sheets-Sheet 1

*Fig. 1.*



INVENTOR

RALPH B. PORTER,

by:

*John E. Jackson*

his Attorney.

Jan. 11, 1944.

R. B. PORTER

2,338,781

# METHOD AND APPARATUS FOR CONTINUOUSLY CASTING METALS

Filed April 24, 1942

2 Sheets-Sheet 2

Fig. 2.



INVENTOR  
RALPH B. PORTER,  
by  
*John E. Jackson*  
his Attorney.

## UNITED STATES PATENT OFFICE

2,338,781

## METHOD AND APPARATUS FOR CONTINUOUSLY CASTING METAL

Ralph B. Porter, Johnstown, Pa.

Application April 24, 1942, Serial No. 440,370

10 Claims. (Cl. 22—57.2)

This invention relates to the continuous casting of metal, and more particularly to the direct formation from molten metal of billets and bars of the desired cross-sectional contour.

It is among the objects of the present invention to reduce as much as possible the number and magnitude of operations necessary to produce metallic billets and bars of relatively small cross-sectional area.

Heretofore there have been proposed a number of methods and apparatus for the continuous casting of molten metal into small ingots, billets, or bars of desired cross-sectional contour (i. e., round, square, oblong, or other shape) and of continuous, and therefore indefinite, length. Such methods and apparatus involve the continuous shaping of the liquid metal into cast forms of desired cross section, and the removal or dissipation of heat from the metal in order to obtain solidification. So far as I am aware, the practices of the prior art have required the use of complex apparatus which is difficult and expensive to maintain, whereby the resultant product has been characterized by high cost of production.

Another difficulty inherent in the practices of the prior art is that the resultant product does not possess the proper surface condition to permit of its being used in sufficient quantity to render operations commercially feasible.

The invention, then, comprises the features hereinafter fully described and as particularly pointed out in the claims, the following description and the annexed drawings setting forth in detail a certain illustrative embodiment of the invention, this being indicative of one of the number of ways in which the principles of the invention may be employed.

In said drawings:

Figure 1 is an elevational view of the apparatus of the present invention, parts thereof being illustrated in section.

Figure 2 is a fragmentary sectional elevation illustrating some of the upper parts of the apparatus, particularly the compression chamber, compacting apparatus, extrusion chamber, mold-forming mandrel, and teeming apparatus.

Figure 3 is a sectional view on the line III—III of Figure 2.

Referring more particularly to the drawings, the numeral 2 designates a horizontal pouring platform from which there depends a substantially vertical cylindrical housing 3 which comprises a compression chamber within which there is continuously formed a refractory mold

of mold sand or other suitable granular material. Such granular mold material may comprise a mixture of foundry sand with the usual binding materials (i. e., flour, bentonite, and molasses). This compression chamber 3 carries in vertical dependency a cylindrical housing 4 of reduced diameter which connects and communicates therewith through a reducing section 5 of inverted frusto-conical shape. The lower cylindrical housing 4 comprises an extrusion chamber from which the refractory mold is continuously ejected in a manner which will be later described. The upper end of the compression chamber 3 is provided with a closure 6 having a central aperture 7 in which there is carried a collar 8. The upper end of this collar 8 has a radial flange 9 which rests upon the closure 6. Disposed to extend through the collar 8 is a cylindrical tube 10 which carries at a position immediately below the closure 6 a radial flange 11, between which and the bottom of the closure 6 is an antifriction bearing 13. Secured to the upper end of the cylindrical tube 10, and resting upon the top of the radial flange 9 of the collar 8 is a bevel gear 15 through the medium of which the cylindrical tube 10 may be rotated.

Referring more particularly to Figure 2, the cylindrical tube 10 extends through the compression chamber 3 and terminates within the reducing section 5. Formed on the periphery of the cylindrical tube 10 is a spiral screw 17.

Granular mold material is introduced to the compression chamber 3 adjacent the top thereof through an aperture 19 which communicates with an outboard hopper 20. According to the foregoing construction and arrangement, it will be seen that the introduction of the granular mold material into the hopper 20 and the rotation of the bevel gear 15 will result in the compacting of the mold material within the compression chamber 3 and the forcing of the said compacted material into and through the reducing section 5 and extruding chamber 4. Preferably the granular mold material must not only be capable of resisting heat, plastic, and porous, but also capable of reuse. In its movement through the reducing section 5 and into the extrusion chamber 4 it is extruded over a mandrel to form a vertical mold into which the molten metal is poured. Accordingly, there is disposed within the cylindrical tube 10 an elongate tube 24 which extends through and projects from the bevel gear 15 and carries on its upper end a conical pouring funnel 25. The lower end of the elongate cylindrical tube 24 projects through, and extends from, the

bottom of the cylindrical tube 10. A cylindrical tube 26 of enlarged diameter is carried on the lower end of the elongate cylindrical tube 24 through the medium of an intermediate enlarging section 27 of frusto-conical shape. The elongate cylindrical tube 24, its conical pouring funnel 25, the larger cylindrical tube 26, and the frusto-conical enlarging section 27 are continuously lined throughout with a refractory material 28 which is capable of withstanding protracted periods of contact with the molten metal to be cast.

It is to be particularly noted that the lower end of the cylindrical tube 24 terminates at the bottom of the reducing section 5 and that the larger cylindrical tube 26 and enlarging section 27 lie within the extruding section 4. Such construction permits the spiral screw 17 to force the granular mold material downwardly through the compression chamber 3 and reducing section 5 before the diametrically larger portions (27-26) at the bottom of the elongate cylindrical tube 24 are encountered. This enables the desired compressing relationship prior to the movement of the compressed or compacted mold material over the diametrically larger portions of the mandrel at the bottom of the elongate cylindrical tube 24. In the manner aforesaid, the lower end of the elongate cylindrical tube 24, the expanding section 27, and the larger cylindrical tube 26 provide a mandrel which affords interior support for the granular mold material being extruded; and the mold, designated hereinafter at X, emerges from the lower end of the extruding chamber 4 with an interiorly formed cylindrical bore which forms the mold cavity or matrix.

Disposed on the pouring platform 2 is a conveyor 29 which is capable of continuously feeding the granular mold material to the hopper 20. Disposed adjacent the conical pouring funnel 25 is a motor 30, and an associated speed reducer 31 having a driven bevel gear 32 which meshes with the bevel gear 15 on the upper end of the cylindrical tube 10. The motor 30 thus continuously rotates the cylindrical tube 10 and the spiral screw 17 within the compression chamber 3, while the granular mold material is continuously teemed into the conical pouring funnel 25 and flows through the refractory lining 28 which extends through the bottom of the cylindrical tube 26 and into the cylindrical matrix provided in the refractory mold X which is continuously extruded from the bottom of the extruding chamber 4. At the beginning of the teeming operation a refractory plug (not shown) is disposed in the cylindrical matrix of the extruded refractory mold X, and as the said refractory mold moves out of the lower end of the extruding chamber 4, molten metal is teemed into the conical pouring funnel 25 at a rate commensurate with the rate of extrusion aforesaid. Thus the mold and billet move in synchronism. The porosity of the extruded mold X permits quick removal of heat from the cast metal, and the outer surfaces of the billet are quickly frozen.

Disposed below the extrusion chamber 4 is a conventional sand stripper 35 which removes the mold X from around the cast billet. Immediately above the sand stripper 35 is a system of water jets 36 which facilitate the stripping operation. The sand or other granular material of which the mold X is composed, after stripping, falls into a collector 37 from which it is moved by a conveyor 38 to the conveyor 29 on the pouring platform 2 which feeds the hopper 20. Disposed below the sand stripper 35 is a pair of re-

tarding rolls 40. These retarding rolls 40 are suitably shaped to accommodate the contour of the solidified billet. Above and below the retarding rolls 40 are suitable water sprays 41 which serve to chill the surfaces of the solidified casting.

It will be understood that as the solidified casting leaves the retarding rolls 40, it may be moved in any direction and given any desired processing treatments. In the embodiment shown, a guide 43 is disposed below the retarding rolls 40, the same being constructed and arranged to divert the downwardly-moving continuous casting into a horizontal path. Immediately beyond the guide 43 is a pair of pinch rolls 44 which direct the horizontally moving continuous casting onto a bed of carrier rolls 45. From the carrier rolls 45 the continuous casting may, for example, be transferred to a shearing mechanism (not shown) which may be used to cut the continuous casting into billets of desired length, after which the said billets may be additionally rolled with or without reheating, as desired.

It will be understood by those skilled in the art that while the continuously extruded refractory mold X and continuously cast billet within the matrix thereof are shown as being of cylindrical shape, they may take other forms such as the round, square, oblong, or other shapes referred to hereinbefore.

The method and apparatus of the present invention may be adapted to the production of billets of tubular form by the simple device of disposing within the conical pouring funnel 25, and to extend throughout the elongate cylindrical tube 24, a suitable mandrel (not shown) the purpose of which is to form the interior wall of the tube. This mandrel may be provided with a slight taper throughout its length to permit shrinkage of the cast metal as it solidifies. Such a mandrel might be of hollow formation and supplied with a cooling fluid introduced from above the cylindrical pouring funnel 25 and carried in interior channels throughout its length and back to a point of exit above the said pouring funnel.

Another modification contemplates the introduction of a lubricant to the inner walls of a compression chamber 3 and extrusion chamber 4. Such a lubricant could be introduced through small apertures (not shown) arranged in a horizontal plane around the said compression chamber. However, when using a molding mixture of suitable consistency, such a lubricant is ordinarily unnecessary.

While I have shown and described several specific embodiments of the present invention, it will be seen that I do not wish to be limited exactly thereto, since various modifications may be made without departing from the scope of the invention as defined in the appended claims.

I claim:

1. The method of continuously casting metal billets and the like, which comprises continuously extruding a hollow bonded granular refractory mold, continuously teeming said mold, permitting the teemed metal to solidify within the continuously extruded mold, and removing the continuously extruded mold from around the continuously cast billet.

2. The method of continuously casting metal billets and the like, which comprises continuously extruding a hollow bonded granular refractory mold, continuously teeming said mold during the extrusion thereof, permitting the teemed metal to solidify within the continuously extruded mold, and removing the continuously

extruded mold from around the continuously cast billet.

3. The method of continuously casting metal billets and the like, which comprises continuously extruding a hollow bonded granular refractory mold, continuously teeming said mold during the extrusion thereof and at a rate which is substantially the same as the rate of extrusion, permitting the teemed metal to solidify within the continuously extruded mold, and removing the continuously extruded mold from around the continuously cast billet.

4. The method of continuously casting metal billets and the like, which comprises continuously extruding a hollow bonded granular refractory mold, continuously teeming said mold, permitting the teemed metal to solidify within the continuously extruded mold, removing the continuously extruded mold from around the continuously cast billet, and chilling the said billet after the mold has been removed therefrom.

5. The method of continuously casting metal billets and the like, which comprises continuously extruding a hollow bonded granular refractory mold, continuously teeming said mold during the extrusion thereof, permitting the teemed metal to solidify within the continuously extruded mold, removing the continuously extruded mold from around the continuously cast billet, and chilling the said billet after the mold has been removed therefrom.

6. The method of continuously casting metal billets and the like, which comprises continuously extruding a hollow bonded granular refractory mold, continuously teeming said mold during the extrusion thereof and at a rate which is substantially the same as the rate of extrusion aforesaid, permitting the teemed metal to solidify within the continuously extruded mold, re-

moving the continuously extruded mold from around the continuously cast billet, and chilling the said billet after the mold has been removed therefrom.

5 7. Apparatus for continuously casting metal billets and the like comprising, in combination, means for continuously extruding a bonded granular refractory mold, means for continuously teeming molten metal into said mold, and means for removing said mold from the cast billet after the solidification thereof.

10 8. Apparatus for continuously casting metal billets and the like comprising, in combination, means for continuously extruding a bonded granular refractory mold, means for continuously teeming molten metal into said mold during the extrusion thereof, and means for removing said mold from the cast billet after the solidification thereof.

15 9. Apparatus for continuously casting metal billets and the like comprising, in combination, means for continuously extruding a bonded granular refractory mold, means for continuously teeming molten metal into said mold, means for removing said mold from the cast billet after the solidification thereof, and means for chilling said billet after the mold has been removed therefrom.

20 25 10. Apparatus for continuously casting metal billets and the like comprising, in combination, means for continuously extruding a bonded granular refractory mold, means for continuously teeming molten metal into said mold during the extrusion thereof, means for removing said mold from the cast billet after the solidification thereof, and means for chilling said billet after the mold has been removed therefrom.

RALPH B. PORTER.